

3,704,122  
**ELECTROPHOTOGRAPHIC PLATE COMPRISING A PHOTOCOCONDUCTOR DISPERSED IN A RESIN BINDER**

Nario Yamaguchi, Sakae Shimizu, and Kazuo Tubuko, Tokyo, Japan, assignors to Kabushiki Kaisha Ricoh, Tokyo, Japan

No Drawing. Continuation of abandoned application Ser. No. 780,282, Nov. 29, 1968. This application June 10, 1971, Ser. No. 151,926

Claims priority, application Japan, Dec. 6, 1967, 42/77,946, 42/77,947; Dec. 12, 1967, 42/79,629; Dec. 23, 1967, 42/82,581; Dec. 27, 1967, 43/83,736

Int. Cl. G03g 5/04

U.S. Cl. 96—1.8

6 Claims

## ABSTRACT OF THE DISCLOSURE

An electrophotographic copying material comprising a support and a light-sensitive or photoconductive layer formed on one surface of said support by a resinous binder, wherein said photoconductive layer contains a photoconductive substance and is formed by a series of steps of (1) dispersing said photoconductive substance in an aqueous emulsion prepared by emulsifying a synthetic film-forming resin or a natural film-forming resin in an aqueous emulsifier solution containing a volatile basic compound and an acidic compound thereafter (2) coating the resultant emulsion containing dispersed photoconductive substance on said support, and then drying the coated support.

This application is a continuation of application Ser. No. 780,282, filed Nov. 29, 1968 and now abandoned.

## BACKGROUND OF THE INVENTION

### Field of the invention

The present invention relates to an electrophotographic copying material comprising a support and a photoconductive layer formed on one surface of said support by a water-emulsified resinous binder.

### Description of the prior art

The electrophotographic copying materials in the prior art were manufactured by a method wherein a metallic plate, or a special paper whose back had been processed to render it electroconductive, was used as a support. A light-sensitive or photoconductive layer-forming solution obtained by dispersing a photoconductive substance in a binder solution, prepared by dissolving a resin in an organic solvent, was applied onto the surface of said support and then dried. In this prior method, however, a water soluble resin was not generally used for said purpose because it does not provide the photoconductive layer formed on the support with the critical electrostatic characteristics—especially, high electric resistance—required for photoconductive layers. Accordingly, it was formerly considered particularly advisable to use a natural or synthetic resin which was soluble only in an organic solvent, and also which would not interfere with the electrostatic characteristics of the photoconductive layer formed on the support. However, in those cases in which a resin that is soluble only in an organic solvent was employed for said purpose, it was necessary to prepare the binder by dispersing the resin in a large quantity of organic solvent because of the general requirement for using a homogeneous dispersion of the photoconductive substance in said binder. As a result, there were various drawbacks in the manufacture of electro-

photographic copying materials in the prior art, such as:

(a) It was conventional to employ expensive organic solvents so that it was necessary to recover these solvents during the manufacturing process.

(b) Most of the organic solvents used are inflammable and involve the risk of explosion, so that preventive measures were required therefor.

(c) Many organic solvents used are hazardous to health, so that protective measures against their effects were also required.

(d) Expensive special measures and coating devices were required to form a photoconductive layer on the support.

(e) Because an air-knife is inoperable as a coating-applying means for such prior compositions, high-speed coating was impractical.

In view of the fact that the above-mentioned disadvantages may be eliminated, if the resin used for the binder is water-emulsive or water-dispersive, there have been proposed a variety of water-emulsive or water-dispersive resins. However, the prior copying materials heretofore produced from these materials had such drawbacks as poor electrostatic characteristics. For example, when an electrostatic charge was impressed on the photoconductive layer by corona discharge, the charged potential become low. Also, the decay of the electric potential, i.e. the dark-decay when said materials were left in a dark place after being charged, was great. Accordingly, such materials have proven to be quite unsatisfactory for practical use.

## SUMMARY OF THE INVENTION

It is, therefore, an object of the invention to provide an electrophotographic copying material which avoids the aforesaid drawbacks of electrophotographic copying materials made with the water-emulsified resinous binders in the prior art.

Another object of the invention is to provide a water-emulsified resinous binder which is suitable for forming a photoconductive layer having superior electrostatic characteristics in an electrophotographic copying material.

It is another object of the invention to provide an electrophotographic copying material which can be produced economically while avoiding the hazards that are encountered in the process of manufacturing said copying material in the prior art.

In brief, the electrophotographic copying material of the present invention is obtained by the following process: a resinous binder having film-forming properties is emulsified with an aqueous emulsifier solution which comprises (1) at least one volatile basic compound selected from the group consisting of nitrogen-containing compounds and (2) at least one acidic compound selected from the group consisting of (a) a natural resin having an electric resistance of at least  $10^{11} \Omega\text{-cm}$ . and containing a resin acid, (b) a synthetic resin having an electric resistance of at least  $10^{11} \Omega\text{-cm}$ . and an acid value, i.e. acid reaction, (c) an alicyclic compound having a carboxyl radical, (d) an aliphatic carboxylic acid, (e) an aromatic carboxylic acid, and (f) acid anhydrides of said carboxylic acids. The emulsion thus obtained has dispersed therein the photoconductive substance. The surface of a support is coated with said dispersion and dried thereafter. Also, in the present invention, there are employed for the aforesaid resinous binder a variety of natural resins as well as synthetic resins having film-forming properties. The emulsion of the resin is produced by using the minimum quantity of organic solvent. Furthermore, the emulsion produced in such a way is characterized by being comprised of the resinous binder in

the form of dispersed fine grains having a diameter of a few  $\mu$ , so that the resultant photoconductive layer is highly homogeneous.

In the present invention, the water-emulsified resinous binder used to form a photoconductive layer is one member selected from the group consisting of the following members (a)-(f).

(a) An emulsion produced by emulsifying a film-forming resinous binder with an aqueous solution of a natural resin containing a resin acid and having an electric resistance of at least  $10^{11} \Omega\text{-cm}$ . and containing a volatile basic compound therein.

(b) An emulsion produced by emulsifying a film-forming resinous binder with an aqueous solution of an alicyclic compound having carboxyl radical and containing a volatile basic compound therein.

(c) An emulsion produced by emulsifying a film-forming resinous binder with an aqueous solution of at least one acid selected from the organic acid group consisting of an aliphatic carboxylic acid, an aromatic carboxylic acid, and an acid anhydride of said carboxylic acids and containing a volatile basic compound.

(d) An emulsion produced by emulsifying a film-forming resinous binder with an aqueous solution of a synthetic resin having an acid value and an electric resistance of at least  $10^{11} \Omega\text{-cm}$ . and containing a volatile basic compound therein.

(e) An emulsion produced by using an organic solution of a synthetic resin such as employed for (d) to supply the film-forming resinous binder and emulsifying the organic solvent solution with an aqueous solution containing a volatile basic compound. In the case of this particular emulsion, the combined use of a small amount of a heavy metal salt of a naphthenic acid as the binder setting agent is preferable.

(f) An emulsion produced by employing, as a film-forming resinous binder, a copolymer selected from the group consisting of a vinyl copolymer having an epoxy radical ( $-\text{O}-$ ), and a vinyl copolymer having a hydroxyl radical ( $-\text{OH}$ ) in its molecular end, and by emulsifying said binder with an aqueous solution of a volatile basic compound and an acid compound such as are applied in (a)-(b).

It is to be noted that, although it is possible to dissolve a resinous binder in an organic solvent and then to emulsify the resultant solution in water by means of an ordinary anionic or nonionic surface active agent, the photoconductive layer formed by employing an emulsion so obtained has too low an electric resistance to provide a sufficient electrostatic light-sensitivity and, therefore, is not of practical use.

As can be seen in the foregoing, in the binders to be applied in the present invention, an aqueous solution of a volatile basic compound is a principal component of the emulsion of the resinous binder. To be more specific, these binders are emulsified by an emulsifier produced by the combination of said volatile basic compound and an acidic compound (such as a natural resin containing a resin acid in the case of (a), a carboxylic acid of an alicyclic compound in the case of (b), an organic acid group in the case of (c), and a synthetic resin having an acid value in the case of (d) as described in the foregoing).

Next, as said volatile basic compound to be employed in the emulsion in the present invention, nitrogen containing compounds, such as ammonia, methylamine, dimethylamine, trimethylamine, ethylamine, diethylamine, triethylamine, propylamine, butylamine, hexylamine, ethylenediamine, arylamine, morpholine, piperidine and hydrazine, are suitable. However, the applicable compounds for said purpose covers also a wide range of amine compounds, which are volatile and water-soluble, such as aliphatic primary amines, secondary amines, and tertiary amines. Besides, in emulsifying resinous binders such as natural resins and synthetic resins which have film-forming

properties, said volatile basic compounds are employed in the form of an aqueous solution.

As the acid compound, i.e. a natural resin containing a resin acid, to be employed for the aforesaid (a), a resin having an electric resistance of at least  $10^{11} \Omega\text{-cm}$ . is selected lest its special quality should be deteriorated when applied in a photoconductive layer. Natural resins having such a property and considered suitable for use include, for example, elemi, Gurjun balsam, jalap, scammonia, amber, bdellium, sagapenum, Euphorbium, myrrh, Opopanax, various kinds of dammar (such as Benak, dead dammar, Melanty, Chan, yon banoun, papuan dammar), shellac, acaroid, dragon brad, mystic, styrax, Canada balsam, Mecca balsam, copaiba balsam, Peru balsam, guaiac, tacamahac, galvanum, gamboge, olibanum, ammoniac, asafetida, various kinds of copal (such as kauri copal, soft manila copal, hard manila copal, congo copal, benguela copal, angora copal, Madagascar copal, Zanzibar copal, demera copal, hard bornea copal, New Zealand kauri copal), various kinds of rosin (such as gum rosin, heterogeneous rosin, polymerized rosin, hydrogenated rosin, tall oil, rosin maleate, rosin oxide, hardened rosin, ester gum), benzoic acid, sandarack, true balsam, and kawakawa resin. Included are various products whose principal component is one of those enumerated above, which have been put on the market under different trade names.

Acid compounds for (b), i.e. carboxylic acids of alicyclic compounds, include, for example, abietic acid, bisnorcholanic acid,  $\beta$ -boswellic acid, chenodesoxycholic acid, chenobic acid, cholic acid, cholic acid, dehydrocholic acid, dioxycoumarin, doisynolic acid, erythrofuscinic acid, etiocholanic acid, glycocholic acid, glychyrhizic acid, oleanolic acid, helvolic acid, hiodesoxycholic acid, isocholic acid, naphthenic acid, norcholanic acid,  $\alpha$ -pimamic acid, quillaic acid, ursodesoxycholic acid, and ursolic acid.

Acid compounds for (c), i.e. an aliphatic carboxylic acid, an aromatic carboxylic acid, and an acid anhydride of said carboxylic acids, include many applicable acids, and examples are enumerated as follows:

Aliphatic saturated monocarboxylic acid: caproic acid, heptanoic acid, caprylic acid, pelargonic acid, capric acid, n-undecylenic acid, lauric acid, n-tridecylenic acid, myristic acid, n-pentadecylenic acid, palmitic acid, margaric acid, stearic acid, n-nonadecylenic acid, arachidic acid, n-heneicosanoic acid, behenic acid, n-tricosanoic acid, lignoceric acid, n-pentacosanoic acid, ceratic acid, n-heptacosanoic acid, montanic acid, n-nonacosanoic acid, melissic acid, n-hentriacontanoic acid, n-dotriacontanoic acid, n-tetracontanoic acid, ceroplastic acid, n-hexatriacontanoic acid, n-octatriacontanoic acid and n-hexatetracontanoic acid.

Aliphatic olefin monocarboxylic acid: 2-hexenoic acid, 3-hexenoic acid, 4-hexenoic acid, 5-hexenoic acid, 2-methyl-2-pentenoic acid, 3-methyl-2-pentenoic acid, 4-methyl-2-pentenoic acid, 4-methylpentenoic acid,  $\alpha$ -ethylcrotonic acid, 2,2-dimethyl-3-butenoic acid, 2-heptenoic acid, 2-octenoic acid, 4-deceneoic acid, 9-deceneoic acid, 9-undecenoic acid, 10-undecenoic acid, 4-dodeceneoic acid, 5-dodeceneoic acid, 4-tetradecenoic acid, 9-tetradecenoic acid, 9-hexadecenoic acid, 2-octadecenoic acid, cis-6-octadecenoic acid, 9-octadecenoic acid, oil acid, elaidic acid, 11-octadecenoic acid, 12-octadecenoic acid, 9-eicosenoic acid, 11-eicosenoic acid, 11-docosenoic acid, 13-docosenoic acid, erucic acid, 15-tetracosenoic acid and mycolipenic acid.

Aliphatic diolefins carboxylic acid: 2,4-hexadienoic acid, diallylacetone, geranium acid and 2,4-decadienoic acid.

Aliphatic higher unsaturated monocarboxylic acid: hexadecatrienoic acid, linoleic acid, linolenic acid, 6,9,12-octadecatrienoic acid, eicosadienoic acid, eicosatrienoic acid, decosadienoic acid, decosatrienoic acid and hexacosadienoic acid.

Aliphatic saturated dicarboxylic acid: adipic acid, pimelic acid, suberic acid, azelaic acid, sebatic acid, undecane dicarboxylic acid, dodecane dicarboxylic acid, brassylic acid and tetradecane dicarboxylic acid.

Aromatic monocarboxylic acid: benzoic acid, o-toluylic acid, m-toluylic acid, p-toluylic acid, dimethylbenzoic acid, o-ethylbenzoic acid, m-ethylbenzoic acid, p-ethylbenzoic acid, 2,3,4-trimethylbenzoic acid, 2,3,5-trimethylbenzoic acid, 2,3,6-trimethylbenzoic acid, 2,4,5-trimethylbenzoic acid, 2,4,6-trimethylbenzoic acid, 3,4,5-trimethylbenzoic acid, cuminic acid, cinnamic acid, o-nitrobenzoic acid, m-nitrobenzoic acid, p-nitrobenzoic acid, 2,4-dinitrobenzoic acid, 3,5-dinitrobenzoic acid, o-chlorobenzoic acid, p-chlorobenzoic acid, o-fluorobenzoic acid, m-fluorobenzoic acid, p-fluorobenzoic acid, o-bromobenzoic acid, m-bromobenzoic acid, p-bromobenzoic acid, o-iodobenzoic acid, m-iodobenzoic acid, p-iodobenzoic acid, 2,3-dichlorobenzoic acid, 2,5-dichlorobenzoic acid, 2,6-dichlorobenzoic acid, 3,4-dichlorobenzoic acid, 3,5-dichlorobenzoic acid, 2,3-dibromobenzoic acid, 2,4-dibromobenzoic acid, 2,5-dibromobenzoic acid, 2,6-dibromobenzoic acid, 3,4-dibromobenzoic acid, 3,5-dibromobenzoic acid, 2,3-diodobenzoic acid, 2,4-diodobenzoic acid, 2,5-diodobenzoic acid, 2,6-diodobenzoic acid, 3,4-diodobenzoic acid, 3,5-diodobenzoic acid, 2-chloro-5-nitrobenzoic acid, 3-chloro-6-nitrobenzoic acid, 2-bromo-5-nitrobenzoic acid, 2-chloro-cinnamic acid, 2-cyanocinnamic acid, 2-naphthoic acid, 5-chloronaphthoic acid,  $\beta$ -naphthoic acid and 5-bromonaphthoic acid.

Aromatic dicarboxylic acid: phthalic acid, isophthalic acid, terephthalic acid, 3-chlorophthalic acid, 4-chlorophthalic acid, 3,6-dichlorophthalic acid, tetrachlorophthalic acid, tetrabromophthalic acid, tetraiodophthalic acid, naphthalic acid, naphthalene-1,2-dicarboxylic acid, naphthalene-1,4-dicarboxylic acid and naphthalene-1,5-dicarboxylic acid.

Aromatic tricarboxylic acid: 1,2,3-hemimellitic acid and 1,2,4-trimellitic acid.

As synthetic resins having an acid value, which can be employed for (d) and (e), a synthetic resin having an electric resistance of at least  $10^{11} \Omega\text{-cm}$ . is selected for the same reasons as in the case of (a) above. Therefore, the suitable synthetic resins include, for example, copolymer resins of acrylic ester, acrylic-alkyd resin, pure alkyd resin, epoxy ester resin, non-drying type pure alkyd resin, rosin-modified alkyd resin, phenol-modified alkyd resin, styrenated alkyd resin, natural resin-modified phenolic resin, natural resin-modified maleic acid resin, natural resin-modified pentaerythritol resin, natural resin-modified fumaric acid resin, and so forth.

In the present invention, in the case of the emulsification of a resinous binder comprising a natural resin or a synthetic resin having film-forming properties as stated below, one or two kinds of acidic compounds having the aforesaid emulsifier component are employed. For the combination of said acidic compound with a volatile basic compound, a mixing ratio of 1 mol of at least one kind of acidic compound to 1-2 mols of at least one kind of basic compound, will effect homogeneous emulsification of a resinous binder in water.

As the resinous binder, although a variety of resins having film-forming properties are applicable, such resins as enumerated hereunder are most suitable for the aforesaid (a)-(d) in the present invention.

(A) Natural resin and natural resin-modified resin: colophony (rosin), modified colophony, dammar resin, ethyl cellulose acetate, hydroxyethyl cellulose acetate, cellulose acetostearate, and ethylcellulose stearate

(B) vinyl polymer and substituted vinyl polymer:

- (I) Photoconductive vinyl polymer: poly-N-vinylcarbazole, N-vinylcarbazole-ethylacrylate copolymer
- (II) Polyvinyl ester: vinylacetate resin, vinylacetate-crotonic acid copolymer, vinylacetate-vinylstearate co-

polymer, polyvinylstearate, vinylacetate-maleic acid copolymer

(III) Vinylchloride polymer or vinylchloride copolymer: polyvinylchloride, vinylchloride-vinylisobutyl ether copolymer, vinylchloride - vinylacetate-vinylalcohol copolymer, vinylchloride-vinylacetate-maleic anhydride copolymer, polyalkylmethacrylate

(IV) Polyvinyl acetal and vinylacetal copolymer: polyvinyl butyral, vinyl butyral-vinylacetate copolymer

(V) Polystyrene or styrene copolymer: polystyrene, styrene-methacrylic acid copolymer, styrene-butadiene copolymer, styrene-dimethylitaconate copolymer

(VI) Polymer of methacrylic ester: polymethacrylic ester, polyalkylmethacrylate, polymethylmethacrylate

(C) Condensed polymer: styrenated alkyd resin, alkyd-modified rosin resin, alkyd-modified phenol resin, epoxy ester resin, pentaerythritol phthalate resin, polycarbonate

(D) Other resins and synthetic gums: poly indene, poly cyclopentadiene, silicone resin, ketone resin, rubber chloride

The resinous binder to be employed for the aforesaid (f) in the present invention includes vinyl copolymer resins obtained by copolymerizing at least one member selected from the vinyl monomer group consisting of, for example, glycidyl acrylate, glycidyl methacrylate, hydroxyethyl methacrylate, hydroxyethyl acrylate, hydroxypropyl methacrylate, hydroxy propyl acrylate, 5-hydroxypentylvinyl ether



with at least one member selected from the monomer group consisting of, for example, styrene, acrylate, methacrylate, acrylonitrile, vinyl chloride, vinylidene chloride, vinyl acetate, acrylic acid, methacrylic acid, crotonic acid, itaconic acid, maleic acid, and fumaric acid.

The materials of the water-emulsified resinous binder to be employed in the present invention are as enumerated above. The materials other than said water-emulsified binder to be employed in forming a photoconductive layer can be any support, photoconductive substance, and sensitizer as conventionally used. As the photoconductive substance, for instance, zinc oxide, titanium oxide, cadmium sulfide, zinc selenide, and so forth may be cited, and above all, zinc oxide and titanium oxide are desirable. As for the sensitizer to be employed, Phthalein dyes such as Fluorescein, Eosin, Erythrosine, and Rose Bengal, Triphenylmethane dyes such as Malachite Green, Crystal Violet, Basic Fuchsin, Methyl Green, Brilliant Green, Bromophenol Blue, and Tetrabromophenol Blue, Cyanine dyes such as Cryptocyanine and Pinacyanol, Heterocyclic dyes such as Acridine Orange, mixed dyes such as Methylene Grey, and furthermore, Alizarine Red S. Alizarine, and Quinizarin may be cited. As for the support, not only a metallic plate but also either paper or a sheet film whose back has been processed for electric conductivity can be employed, but it is desirable that the surface electroresistivity resulting from said process for electric conductivity be less than  $10^9 \Omega\text{-cm}$ . and it is further advisable for it to be less than  $10^7 \Omega\text{-cm}$ .

A desirable impregnation of the aforesaid sensitizer in a photoconductive layer can be attained by mixing the sensitizer within the range of 0.01-5.0% per total weight of zinc oxide, for example, to be contained in the photoconductive layer.

The copying material of the present invention is produced by the steps comprising: one member selected from the group consisting of emulsion members (a)-(f) as described above is dispersed with a photoconductive substance; the emulsion wherein said photoconductive substance is dispersed is applied as a coating to the surface of a support, by such methods as the centrifugal coating method, spray coating method and brush coating method. The surface thus coated with said emulsion is

dried thereafter. It is noted, in this respect, that according to the present invention, in the manufacturing process of the electrophotographic copying material, the coated surface of the support, that is to say, the photoconductive layer, is impregnated with a volatile basic compound, so that it is necessary to provide a sufficient temperature for volatilization of said basic compound to expedite the drying of the layer. Therefore, it is desirable to take such measures as a hot-air drying method or infrared ray drying method for the sake of rapid drying. As for the drying temperature, though it may depend on the kind of the volatile basic compound employed, the most desirable drying temperature is not lower than 100° C. and also comes within the range of such temperatures as will not cause the resin contained in the photoconductive layer to deteriorate and thereby interfere with its character. The maximum temperature is ordinarily 250° C.

There will be no inconvenience even if there remains a volatile basic compound, in the formed photoconductive layer, in an amount not exceeding 0.5% per total weight of the solid matter (i.e. said photoconductive layer).

Among the electrophotographic copying materials, the copying material having a photoconductive layer formed by the aforesaid (f) member is especially endowed with an excellent character. In other words, an epoxy radical or hydroxyl radical contained in a resinous binder shows a bridge-formation reaction in the drying process for formation of a photoconductive layer and thereby forms a network structure, so that the layer thus formed has outstanding weather-proofness. For instance, even when it is used for copying purposes in an atmosphere of high humidity, the copied picture as well as the characteristic obtained thereby is by no means inferior to those obtained in an atmosphere of normal humidity. This is attributable to the fact that a network structure formed by the resinous binder in the photoconductive layer impedes the adsorption of moisture from the atmosphere by the photoconductive substance. It is further noted that, in the aforesaid drying process, a bridge-formation reaction is readily expedited by the existence of a dibasic acid, a tertiary ammonium salt, and a quaternary ammonium salt in case of an epoxy radical; while in case of a hydroxyl radical at the end of a long-chain molecule it is expedited by the presence of a polybasic acid of an amino resin, and the like. Accordingly, a binder which has such a radical, an acid and a salt cause a bridge-formation reaction at the time of forming a photoconductive layer on the surface of a support as seen above.

#### DETAILED DESCRIPTION OF THE INVENTION

##### Example 1

3 gms. of Stabelite Resin (trade name of a product of Hercules Co. of U.S., having hydrogenated rosin as its principal component and containing abietic acid as a resin acid) is added to 70 gms. of a xylene solution of 70% silicone resin (manufactured by Shinetsu Kagaku Kogyo Kabushiki Kaisha in Japan, and named Silicone Resin KR-211), and then the mixture thus obtained is heated at 70° C. The substance thus treated is emulsified by adding steadily a solution obtained by dissolving 3 gms. of triethylamine in 100 gms. of water, while being agitated by a homomixer.

Meanwhile, another solution is prepared by adding 100 gms. of photoconductive zinc oxide to 100 gms. of water and then dispersing same by a homomixer, and this solution is blended with 80 gms. of the aforesaid emulsion and then agitated. Next, the solution thus processed is further blended with 5 cc. of a methanol solution comprising Bromophenol Blue 1%, Fluorescein 0.5%, and Rose Bengal 0.1%, and agitated.

The photoconductive layer forming solution thus obtained is applied to coat the surface of an art paper, whose back has been processed for electric conductivity, to such

an extent that the weight after the drying process will be 25 gms./m.<sup>2</sup>, and thereafter is dried by the infrared-ray drying method.

A picture, which is obtained by employing such an electrophotographic copying paper impressed with electric charge by an ordinary method and through either wet-process development or dry-process development subsequent to its exposure, is superb in the light of the fact that no such picture has ever been obtained using a copying paper produced by forming a photoconductive layer by the employment of a resinous binder emulsified with an ordinary surface active agent.

##### Example 2

15 When 100 gms. of Styrezol 4440 (50%-mineral turpentine solution of styrenated alkyd resin, manufactured by Dai Nippon Ink and Chemical Inc.) was employed in lieu of KR-211, which was employed in Example 1 above, while otherwise following the processes as that in Example 1 for preparing an electrophotographic copying paper and producing a picture by an ordinary electrophotographic means, the resulting picture was superb.

##### Example 3

25 3 gms. of Dammar Gum (manufactured by Arakawa Rinsan Kagaku Kogyo Kabushiki Kaisha, and having dammarol acid as a resin acid component) is added as in Example 1 and the mixture is heated up to a temperature within the range of 70-80° C. to effect dissolution thereof. The solution thus obtained is agitated by a homomixer, while another solution prepared by dissolving 3 gms. of ethylamine in 100 gms. of water is added steadily, and is thereby emulsified.

30 80 gms. of the resultant emulsion is added to the zinc oxide dispersed solution, as prepared in the above Example 1, and is agitated. A sensitizing dye solution is also added in the same way as in Example 1 in producing the photoconductive layer forming solution.

The employment of the aforesaid processes in producing a picture in the same way as in Example 1 has resulted in a superb picture.

##### Example 4

45 In this case, 4 gms. of Ester Gum (Product of Hercules Co. in U.S., having abietic acid as a resin acid component) is added to 100 gms. of Styrezol 4440, and the mixture is heated up to a temperature within the range of 70-80° C. to effect dissolution thereof. The solution thus obtained is agitated by a homomixer, while another solution prepared by dissolving 4 gms. of triethylamine in 100 gms. of water is added steadily, and is thereby emulsified. 80 gms. of the resultant emulsion is added to the zinc oxide dispersed solution, as prepared in Example 1, and agitated. A sensitizing dye solution is also added in the same way as in Example 1 in producing a photoconductive layer forming solution.

55 When an electrophotographic copying paper, which had been prepared in the same way as in Example 1, was employed in producing a picture by an ordinary process, the resultant picture was superb in quality.

##### Example 5

60 In this case, 2 gms. of Shellac (product of Japan Shellac Industrial Co., Ltd., containing aleuritic acid as its principal component) is added to 80 gms. of Beckozole 1341 (a 60%-Xylene Naphtha solution of phenolized alkyd resin, manufactured by Dai Nippon Ink and Chemicals Inc.), and the mixture thus obtained is heated up to a temperature within the range of 70-80° C. to effect dissolution thereof. The solution thus obtained is agitated by a homomixer, while another solution prepared by dissolving 8 gms. of 28% aqueous ammonia in 100 gms. of water is added steadily, and is thereby emulsified. On the other hand, another solution is prepared by adding 100 gms. of photoconductive zinc oxide into 100

gms. of water and then dispersing same by a homomixer, and thereafter 90 gms. of the aforesaid emulsion is added to this dispersed solution and agitated. The mixture thus obtained is further blended with 6 cc. of a methanol solution containing 2% Rose Bengal.

The photoconductive layer forming solution thus obtained is applied to the surface of a baryta paper, whose back has been processed for electric conductivity, to such an extent that the weight subsequent to the drying process will be 35 gms./m.<sup>2</sup>, and thereafter is dried.

An electrophotographic copying paper obtained as above is impressed with an electric charge by an ordinary method, and can be developed and fixed by dry-process development subsequent to exposure. This material produces a superb photographic effect, so that the picture obtained thereby may be used as a master for offset printing after making it hydrophilic.

#### Example 6

In this case, 3 gms. of Polymer Rosin (product of Hercules Co. in U.S., having abietic acid as a resin acid component) is added to 100 gms. of Beckozole P-787 (a 45%-xylene solution of epoxide ester, manufactured by Dai Nippon Ink and Chemicals Inc.), and the mixture is heated up to a temperature within the range of 70-80° C. to effect dissolution thereof. The solution thus obtained is agitated by a homomixer, while another solution prepared by dissolving 3 gms. of morpholine in 100 gms. of water is added steadily, and is thereby emulsified.

Next, 100 gms. of the resultant emulsion is added into the zinc oxide dispersed solution, as prepared in Example 1 above, and is agitated. A sensitizing dye solution is also added in the same way as in Example 1.

The photoconductive layer forming solution thus obtained is applied for coating the surface of an art paper, whose back has been processed for conductivity, to such an extent that the weight after the drying process will be 25 gms./m.<sup>2</sup>, and is dried thereafter.

This copying material, when used for producing a picture thereon by an ordinary electrophotographic process, has brought about a superb effect.

#### Example 7

In this case, 3 gms. of naphthenic acid is added to 100 gms. of Styrezol 4440, and the mixture is agitated by a homomixer, while a solution prepared by dissolving 3 gms. of morpholine in 100 gms. of water is added steadily, and is thereby emulsified. (The emulsion thus obtained is hereinafter referred to as the A solution.)

On the other hand, 100 gms. of photoconductive zinc oxide is added to 100 gms. of water and dispersed by a homomixer. The dispersed solution thus obtained is blended with 5 cc. of a methanol solution comprising Bromophenol Blue 1%, Fluorescein 0.5%, and Rose Bengal 0.1%, and is agitated. (The solution thus obtained is hereinafter referred to as the B solution.)

The aforesaid B solution is blended with 80 gms. of the A solution and then is agitated. The conductive layer forming solution obtained by the above process is applied for coating the surface of an art paper, whose back has been processed for electric conductivity, to such an extent that the weight after the drying process will be 25 gms./m.<sup>2</sup>, and is dried thereafter.

The resultant electrophotographic copying material, when impressed with an electric charge by a conventional method and developed by the wet-process or the dry-process, produced a superb picture in contrast to the fact that no such a picture has even been obtained by the employment of an emulsion produced by any conventional surface active agent.

#### Example 8

In this case, 1 gr. of abietic acid is added to 70 gms. of KR-211 to be dissolved therein. The solution thus obtained is agitated by a homomixer, while another solu-

tion prepared by dissolving 2 gms. of triethylamine in 100 gms. of water is added thereto steadily, and is thereby emulsified.

80 gms. of the resultant emulsion is then blended with the B solution referred to in the foregoing Example 7, and is agitated. By the employment of the photoconductive layer forming solution thus obtained, an electrophotographic copying paper is produced in the same way as in Example 7. The electrophotographic copying paper thus produced, when employed for producing a picture through a conventional electrophotographic process, has brought about a superb result.

#### Example 9

In this case, except for the employment of 28 gms. of etiocholanic acid in lieu of abietic acid employed in Example 2, the same steps are applied in producing an electrophotographic copying paper. As for the photographic efficiency of the resultant copying paper, the same effect as in Example 1 is attained through the same conventional processes.

#### Example 10

In this case, 3 gms. of oleanolic acid is added to 80 gms. of Beckozole 1341 (a 60% xylene naphtha solution of phenol-modified alkyd resin, manufactured by Dai Nippon Ink and Chemicals Inc.) and dissolved therein. The solution thus obtained is agitated by a homomixer, while another solution prepared by dissolving 3 gms. of morpholine in 100 gms. of water is added steadily, and is thereby emulsified.

90 gms. of the resultant emulsion is then blended with the B solution referred to in the aforesaid Example 7, and is agitated. By the employment of the photoconductive layer forming solution thus obtained, an electrophotographic copying paper is produced in the same way as in Example 7. The electrophotographic copying material thus produced, when employed for producing a picture through a conventional electrophotographic process, has brought about a superb result.

#### Example 11

In this case, 3 gms. of naphthenic acid is added to 110 gms. of Beckozole P-787. The mixture thus obtained is agitated by a homomixer, while another solution prepared by dissolving 3 gms. of triethylamine in 100 gms. of water is added steadily, and is thereby emulsified. On the other hand, 100 gms. of photoconductive zinc oxide is added to 100 gms. of water and dispersed by a homomixer. The dispersed solution thus obtained is mixed with 100 gms. of the aforesaid emulsion and is agitated. Next, 6 cc. of methanol solution containing 2% of Rose Bengal is added, and this mixture is further agitated. The photoconductive layer forming solution thus produced is applied for coating the surface of a baryta paper, whose back has been processed for conductivity, to such an extent that its weight after the drying process will be 35 gms./m.<sup>2</sup>, and is dried thereafter.

The resultant electrophotographic copying material is impressed with an electric charge by a conventional method, and can be developed and fixed by the dry-process subsequent to exposure. This material produces a superb photographic image, so that a picture obtained thereby can be used as a master for an offset printing after making it hydrophilic.

#### Example 12

In this case, 2 gms. of lauric acid was added to 110 gms. of Beckozole P-787. The mixture thus obtained was agitated by a homomixer while another solution, which had been prepared by dissolving 3 gms. of triethylamine in 100 gms. of water, is added steadily, and thereby a binder solution comprising an emulsion of said resin was produced. 110 gms. of the thus produced binder solution was then added to a sensitizer solution comprising 100 gms. of photoconductive zinc oxide, 100 gms. of water, and 5

cc. of a sensitizer solution (a methanol solution consisting of 1% of Bromophenol Blue, 0.5% of Fluorescein, and 0.1% Rose Bengal) and agitated, thereby producing a photoconductive-layer forming solution. The dispersed solution thus prepared was applied for coating the surface of a support—in the present case, an art paper—whose back had been processed for conductivity, to such an extent that the remainder of the applied solution on said surface subsequent to the drying process will be 25 gms./m.<sup>2</sup>. Upon drying said coated support at 130° C. for 1 min., an electrophotographic copying material was obtained.

On the other hand, for the purpose of comparison, another binder solution having the same composition as that of the aforesaid binder solution, except for substitution of 3 gms. of a surface active agent (such as Nissan Rapizole (dialkylsulfosuccinate manufactured by Nihon Yushi Kabushiki Kaisha)) for the lauric acid and triethylamine, was prepared and the same sensitizer solution as in the present invention described in the foregoing was added thereto, and the thus blended solution was further processed in the same way as in the present invention, thereby producing a copying material to serve for said comparison.

When both of those copying materials which were obtained through the aforesaid processes were impressed with an electric charge by corona discharge, the material produced by the present invention showed an electric charge as high as 400 volts, while the other prepared for comparison could be charged with only 50 volts. Moreover, when each of said copying materials was exposed in accordance with an original copy and developed by the wet-process, the material produced by the present invention formed a clear image of the original copy with high fidelity, while the other prepared for comparison could hardly form any image.

#### Example 13

In this case, except for the substitution of palmitic acid for the lauric acid employed for emulsification in the foregoing Example 12, the same components and processes as in case of Example 12 were applied in obtaining an electrophotographic copying material. The efficiency and performance of the thus obtained copying material were equivalent to that of Example 12.

#### Example 14

In this case, 3 gms. of stearic acid was added to 100 gms. of Styrezol 4440. The mixture thus obtained was agitated by a homomixer while another solution, which had been prepared by adding 3 gms. of morpholine to 100 gms. of water, was added steadily, and thereby a binder solution comprising an emulsion of said resin was produced. 100 gms. of the thus produced binder solution was then added to a sensitizer solution having the same composition as that of Example 12, and the thus blended solution was thereafter processed in the same way as in Example 12, thereby producing an electrophotographic copying material. The efficiency and performance of the thus obtained copying material were equivalent to that of Example 12 of the present invention.

#### Example 15

In this case, 3 gms. of oleic acid was added to 70 gms. of Silicone Resin KR-211. The mixture thus obtained was agitated by a homomixer while another solution, which had been prepared by dissolving 3 gms. of triethylamine in 100 gms. of water, is added steadily, and thereby a binder solution comprising an emulsion of said resin was produced. 80 gms. of the thus produced binder solution was then added to a sensitizer solution having the same composition as that of Example 12, and the thus blended solution was thereafter processed in the same way as in Example 12, thereby producing an electrophotographic copying material. The efficiency and per-

formance of the thus obtained sensitive material proved to be equivalent to that of Example 12 of the present invention.

#### Example 16

In this case, 3 gms. of ricinoleic acid was added to 80 gms. of Beckozole 1341. The mixture thus obtained was agitated by a homomixer while another solution, which had been prepared by blending 10 gms. of 28%-ammonia water with 100 gms. of water, was added steadily, and thereby a binder solution comprising an emulsion of said resin was produced. 90 gms. of the thus produced binder solution was then added to a sensitizer solution having the same composition as that of Example 12, and the resultant solution was processed in the same way as in Example 12, thereby producing an electrophotographic copying material. The copying material thus produced proved to be equivalent to that of Example 12 in its efficiency as well as performance.

#### Example 17

In this case, there were prepared several binders: A binder, which was obtained by emulsifying the same silicone resin as was employed in Example 15 by means of an emulsifier produced by combining phthalic anhydride with triethylamine,

A binder, which was obtained by emulsifying the same styrenated alkyd resin as was employed in Example 14 by means of an emulsifier produced through combination of cobalt naphthenate (a hardener), p-chlorobenzoic acid, and trimethylamine,

A binder, which was obtained by emulsifying the aforesaid silicone resin by means of an emulsifier produced by combining naphthalic acid with triethylamine,

A binder, which was obtained by emulsifying the aforesaid silicone resin by means of an emulsifier produced by combining tetrachlorophthalic acid with triethylamine, and

A binder, which was obtained by emulsifying the aforesaid styrenated alkyd resin by an emulsifier produced by combining tetrachlorophthalic acid with trimethylamine.

By the employment of each of the binders enumerated above, and by applying the method of treatment similar to that employed in Example 12, electrophotographic copying materials were produced respectively. Each of the resultant copying materials proved to be equivalent to that of Example 12 in its efficiency and performance.

#### Example 18

In this case, 10 gms. of Styrezol J-718 (a 50%-high solvency mineral turpentine solution of styrenated alkyd resin, whose acid value is approximately 10, manufactured by Dai Nippon Ink and Chemicals Inc.) was added to 100 gms. of Styrezol 4440, and the mixture thus obtained was agitated by a homomixer while another solution, which had been prepared by dissolving 3 gms. of triethylamine in 100 gms. of water, was added steadily, and thereby a binder solution comprising an emulsion of the aforesaid Styrezol 4440 resin was produced. On the other hand, 100 gms. of photoconductive zinc oxide was added to 100 gms. of water, and furthermore, while this mixture was agitated by a homomixer, 5 cc. of a sensitizing dye solution (a methanol solution comprising 1% of Bromophenol Blue, 0.5% of Fluorescein, and 0.1% of Rose Bengal) was added, and thereby a photoconductive substance, that is, a sensitizer dispersed solution, was produced. Next, 80 gms. of the aforesaid binder solution was added to said dispersed solution and, through thorough agitation, a photoconductive-layer forming solution was produced. Subsequently, by application of this solution and also following the same processes for forming a photoconductive layer as employed in Example 1, an electrophotographic copying material was obtained.

## 13

Meanwhile, for the purpose of comparing the efficiency and performance of the copying material obtained in the present invention, another binder was prepared by emulsifying the aforesaid resin by means of such a conventional surface active agent that will scarcely be volatilized even by drying, and by application of said binder, and through the same processes as in the present invention, an electrophotographic copying material was also prepared to serve for the test comparison.

When both of the aforesaid copying materials were impressed with an electric charge through a conventional process, exposed, and then developed by either the wet-process or the dry-process, the copying material which was produced in accordance with the present invention formed a clear image, whether developed by the wet-process or the dry-process, while the other one employed for comparison could hardly form any image regardless of the process of development.

## Example 19

In this case, 15 gms. of Beckozole 1341 was added to 70 gms. of Silicone Resin KR-211, and the mixture thus obtained was agitated by a homomixer while another solution, which had been prepared by dissolving 5 gms. of morpholine in 100 gms. of water, was added steadily, and thereby a binder solution comprising an emulsion of said Silicone Resin KR-211 was produced. Then, 80 gms. of the thus obtained binder solution was added to a photoconductive substance, that is, a sensitizer dispersed solution having the same composition as that of Example 18, and was blended thoroughly by agitation, thereby producing a photoconductive layer forming solution. Subsequently, said solution was used in the same way as in Example 18, and an electrophotographic copying material was obtained thereby. The resultant copying material, when employed for the photographic reproduction by following the same processes as in Example 18, produced quite a clear copied image.

## Example 20

In this case, 10 gms. of 70%-mineral turpentine solution of Super Beckozole 1351 (a pure alkyd resin whose acid value is approximately 20, manufactured by Dai Nippon Ink and Chemicals Inc.) was added to 70 gms. of a xylene solution of Silicone Resin (KR-211) which is the same as that of Example 19, and the mixture thus obtained was agitated by a homomixer while another solution, which had been prepared by dissolving 3 gms. of triethylamine in 100 gms. of water, was added steadily, and thereby a binder solution comprising an emulsion of said Silicone Resin KR-211 was produced. Subsequently, 80 gms. of the thus obtained binder solution was processed for application in the same way as in Example 18, and an electrophotographic copying material was produced thereby.

## Example 21

In this case, except for substitution of 15 gms. of 50%-toluene solution of Aron S-1001 (trade name of product of Toa Gosei Kagaku Kogyo Kabushiki Kaisha, whose acid value is approximately 12) which is a copolymer resin whose principal component is an acrylic ester, for the solution of a pure alkyd resin employed in the foregoing Example 20, the same components and processes of treatment as in Example 20 were applied in obtaining an electrophotographic copying material. The efficiency and performance of the resultant copying material were equivalent to that of Example 20.

## Example 22

In this case, except for substitution of 15 gms. of solution of a styrenated alkyd resin (i.e. the same as employed in Example 18) for the solution of a pure alkyd resin employed in Example 20, the same components and processes of treatment were applied in obtaining an elec-

## 14

trophotographic copying material. The efficiency and performance of the resultant copying material were equivalent to that of Example 20.

## Example 23

In this case, except for the substitution of 10 gms. of 50%-xylene and butanol solution of Lustrazol A-401 (a manufacture of Dai Nippon Ink and Chemicals Inc., whose acid value is approximately 5), which is a copolymer resin whose principal component is an acrylic ester, for the solution of pure alkyd resin employed in the aforesaid Example 20, the same components and processes of treatment were applied in obtaining an electrophotographic copying material. The efficiency and performance of the resultant copying material were equivalent to that of Example 20.

## Example 24

In this case, 0.5 gr. of manganese naphthenate (a hardener) was added to 100 gms. of a mineral turpentine solution of a styrenated alkyd resin (i.e. the same as employed in Example 18), and this mixture was agitated by a homomixer while another solution, which had been prepared by dissolving 3 gms. of triethylamine in 100 gms. of water, was added steadily, and thereby a binder solution comprising an emulsion of said resin was produced. On the other hand, 0.25 gr. of manganese naphthenate and 0.25 gr. of cobalt naphthenate were added to 100 gms. (50 gms. solid) of a mineral turpentine solution of rosin-modified alkyd resin (manufactured by Japan Reichhold Chemicals Inc.), and this mixture was agitated by a homomixer while another solution, which had been prepared by dissolving 2 gms. of triethylamine and 1 gr. of trimethylamine in 100 gms. of water, was added thereto, and was thereby emulsified. Subsequently, 100 gms. each of the binder solutions thus emulsified was respectively added to a photoconductive substance, that is, a sensitizer dispersed solution having the same composition as that of the aforesaid Example 18, and blended thoroughly by agitation, thereby producing two types of photoconductive layer forming solutions. Then, said solutions were respectively treated in the same way as in Example 18, and electrophotographic copying materials were obtained thereby. The resultant copying materials when employed for copying, have proved equivalent to that of Example 18 in their efficiency and performance.

## Example 25

In this case, 600 gms. of toluene, 270 gms. of styrene, 200 gms. of butyl methacrylate, 60 gms. of  $\gamma$ -hydroxypropylmethacrylate, 20 gms. of itaconic acid, and 12 gms. of azobisisobutyronitrile were put together in a three neck flask, and upon replacing the air within said flask by nitrogen, said mixture was polymerized over a period of 5 hours by heating at 100° C., and thereby a copolymerized resinous binder (hereinafter referred to as copolymer A) was obtained.

Next, 3 gms. of naphthenic acid was added to 100 gms. of said copolymer A, and this mixture was agitated by a homomixer while 100 gms. of 3%-aqueous solution of triethylamine was added steadily, and thereby a binder solution comprising an emulsion of said copolymer A was produced.

Then, 100 gms. of photoconductive zinc oxide, 100 gms. of water, and 1 gr. of tartaric acid were added to 80 gms. of said emulsified binder, and the mixture thus obtained was further agitated by a homomixer for 10 min. Subsequently, 3 cc of a sensitizer solution (a methanol solution comprising 1% of Bromophenol Blue and 0.5% of Rose Bengal) was added to the resultant solution, and a photosensitive-layer forming solution was produced thereby. The photosensitive-layer forming solution thus produced was applied for coating the surface of an art paper, whose back had been processed for conductivity, to such an extent that the remainder of the applied

sensitizer on said surface subsequent to the drying process was 30 gms./m.<sup>2</sup>. Then, the thus coated support was dried at 120° C. for 10 min. and thereafter left in a dark place (temp. 20° C., RH 65%) for modulation of the humidity for 24 hours, and thereby an electrophotographic copying material was obtained.

On the other hand, for the sake of comparison, another copying material was prepared by means of employing a copolymer which was composed by merely omitting the  $\gamma$ -hydroxypropylmethacrylate from the components of the aforesaid polymer A, while processing it in the same way as was employed above. (Said copying material thus obtained for the sake of comparison is hereinafter referred to as compared material a.) Also, for the same purpose of comparison, one more sample of copying material was also prepared by means of employing an emulsified binder obtained by emulsifying the aforesaid copolymer A by use of sodium alkylbenzenesulfonate, while processing it in the same way as was employed in the present invention. (Said copying material thus obtained for the sake of comparison is hereinafter referred to as compared material b.)

Subsequently, evaluation of each of the foregoing copying materials was conducted with regard to their electrostatic characteristics as shown below:

Electric chargeability: Surface electric potential 30 sec. after the impression of an electric charge on the sensitive layer by corona discharge ( $V_s$ ).

Dark decay: By estimating the electric potential 5 sec. after the stopping of the corona discharge to be  $V_{35}$ , and the electric potential 30 sec. after the stopping of corona discharge to be  $V_0$ , the value is calculated by the formula

$$\frac{V_{35} - V_0}{V_{35}} \times 100$$

Sensitivity: The quantity of light irradiation required for lowering the aforesaid electric potential  $V_0$  to 10% thereof (lux/sec.).

The results of evaluations conducted on the respective characteristics of the aforesaid materials were as shown in the following Table 1.

TABLE 1

| Copying material              | Electric chargeability<br>$V_s(V/\mu)$ | Dark decay<br>(percent) | Sensitivity<br>(lux/sec.) |
|-------------------------------|----------------------------------------|-------------------------|---------------------------|
| Material of present invention | 40                                     | 10                      | 320                       |
| Compared material a           | 35                                     | 30                      | 360                       |
| Compared material b           | 5                                      | 100                     | -----                     |

Furthermore, as a result of putting the respective copying materials into practical use for the formation of copies, it was found that the material of the present invention was quite superior to the compared material a while the compared material b was conspicuously inferior to the compared material a in terms of the concentration of image and clearness of the produced copy.

#### Example 26

In this case, except for containing the same amount of  $\beta$ -hydroxyethylmethacrylate in lieu of  $\gamma$ -hydroxypropylmethacrylate, a copolymer having the same composition as the copolymer A in the foregoing Example 25 was prepared. This copolymer is hereinafter referred to as copolymer B. Then, said copolymer b was processed in the same way as in Example 25, and thereby an electrophotographic copying material was obtained.

On the other hand, for the sake of comparison of efficiency, another copolymer comprising the components of the aforesaid copolymer B, excluding the  $\beta$ -hydroxyethylmethacrylate, was prepared through the same processes as employed in the present invention, and thereby a copying material to serve for comparison was produced.

As a result of comparison of the efficiency and performance in terms of the concentration of image and clearness of produced copy as well as electrostatic characteristics of these copying materials, it was found that the material of the present invention was far superior to said comparison material.

#### Example 27

In this case,  $\gamma$ -hydroxypropylmethacrylate of the copolymer A in Example 25 was replaced with the same weight of  $\beta$ -hydroxyethylmethacrylate, while the composition ratio of other monomers was left the same. Into 100 gms. of the copolymer thus prepared (hereinafter referred to as copolymer C) was added 3 gms. of phthalic acid, and this mixture was thoroughly agitated by a homomixer while 3% aqueous solution of trimethylamine was added steadily, to emulsify and produce a binder thereby.

Subsequently, 100 gms. of photoconductive zinc oxide, 100 gms. of water, and 3 cc. of sensitizing dye (the same composition as in Example 1) were added to 80 gms. of the thus emulsified binder solution, and agitated by a homomixer for 10 min. Then, by employing the processes and a support the same as that used in Example 25, an electrophotographic copying material was obtained.

On the other hand, another copolymer was produced by excluding  $\beta$ -hydroxyethylmethacrylate from said copolymer C while leaving the composition ratio of the other monomers the same, and following the same steps as in the present invention, so as to provide a copying material for the purpose of comparison. Then, evaluation of the electrostatic characteristics of each of the aforesaid copying materials was conducted by the same method as in Example 25. The values thus determined are shown in the following Table 2.

TABLE 2

| Copying material                 | Electric chargeability<br>$V_s(V/\mu)$ | Dark decay<br>(percent) | Sensitivity<br>(lux/sec.) |
|----------------------------------|----------------------------------------|-------------------------|---------------------------|
| Material under present invention | 42                                     | 12                      | 310                       |
| Compared material                | 46                                     | 32                      | 370                       |

In case of the copying material in the present invention, it is understood that, either in the course of the drying or while in the state of being heated subsequent to the drying of the sensitive solution applied to the surface of a support, trimethylamine contained in said solution was volatilized, and a carboxylic acid such as itaconic acid or phthalic acid and the  $-OH$  radical of  $\beta$ -hydroxyethylmethacrylate caused a bridging-reaction, and accordingly, the copying material of the present invention proved satisfactory in respect of its electrostatic characteristics as well as its copying performance as compared with those materials employed for comparison.

#### Example 28

In this case, a composition of monomers comprising 500 gms. of toluene, 200 gms. of styrene, 150 gms. of butyl methacrylate, 50 gms. of ethyl acrylate, 58 gms. of acrylonitrile, 40 gms. of glycidylmethacrylate, 2 gms. of acrylic acid, and 8 gms. of benzoyl peroxide was slowly agitated within a three neck flask, in which air had been replaced by nitrogen, while being heated at 90° C. for a 6-hour polymerization. Subsequently, the thus polymerized product was cooled, and a 50% solid copolymer was obtained thereby. (This material is hereinafter referred to as copolymer D.)

Next, 10 gms. of Styrezol 4440 and 3 gms. of phthalic anhydride were added to 100 gms. of said copolymer D. The mixture thus obtained was agitated by a homomixer while 100 gms. of 3% aqueous solution of isopropylamine [ $(CH_3)_2CHNH_2$ ] was added steadily, and was emulsified.

Then, 100 gms. of zinc oxide powder, 100 gms. of water, and 4 cc. of sensitizing dye (i.e. a methanol solution comprising 0.5% of Bromophenol Blue and 0.5% of

Rose Bengal) were added to 80 gms. of said emulsion. This mixture was intensely agitated for blending for 10 min., and a photosensitive-layer forming solution was thus obtained.

Meanwhile, the employment of an aqueous solution of a polymer comprising an inorganic salt such as sodium chloride or lithium chloride, the back of an art paper was processed for electric conductivity. The surface of the thus processed art paper was then coated with the aforesaid photoconductive-layer forming solution to such an extent that the residue of coating substance (i.e. sensitizer) after drying will be 30 gms./m.<sup>2</sup>. The art paper thus coated was dried at 120° C. for 10 min. and thereafter left hung in a dark place (temp. 20° C., RH 65%) for 12 hours for modulation of humidity, and hereby an electrophotographic copying material was obtained.

On the other hand, for the purpose of comparison, another copying material was produced by employing a copolymer which was composed by merely omitting glycidylmethacrylate from the components of the aforesaid copolymer D, while processing it in the same way as in the present invention.

A subsequent careful comparison in respect of the electrostatic characteristics as well as the actual electrophotographic copying performance revealed that the electric charge of the copying material in the present invention is higher than that of the aforesaid material provided for comparison, and that the degree of dark decay of the former is lower than that of the latter. It has also been confirmed that the former is conspicuously superior to the latter in the image formability and the concentration of image. Moreover, it was observed that such a copying material as produced by employing an emulsion prepared by emulsifying the aforesaid copolymer D by means of a surface active agent such as nonionic, cationic, anionic, or amphoteric ion surface active agent was either utterly ineffective in image-formation or could produce only an unclear image (whose concentration was in the range of 0.2-0.4).

The embodiments of the invention in which an exclusive property or privilege is claimed are defined as follows:

1. The method of preparing an electrophotographic copying material comprising an electroconductive support having a photoconductive film layer on one surface thereof, the said material being capable of assuming and retaining an image-forming electrostatic charge, which method comprises forming an aqueous emulsion of a resinous binder and containing dispersed therein a finely divided photoconductive material, by emulsifying a resinous binder of a copolymer consisting of at least one member selected from the vinyl monomer group consisting of glycidyl acrylate, glycidyl methacrylate, hydroxyethyl methacrylate, hydroxyethyl acrylate, hydroxypropyl methacrylate, hydroxypropyl acrylate, 5-hydroxypentylvinyl ether ( $\text{CH}_2=\text{CHOCH}_2\text{CH}_2\text{CH}_2\text{CH}_2\text{CH}_2\text{OH}$ ) with at least one member selected from the monomer group consisting of styrene, alkyl acrylate, alkyl methacrylate, acrylonitrile, vinyl chloride, vinylidene chloride, vinyl acetate, acrylic acid, methacrylic acid, crotonic acid, itaconic acid, maleic acid and fumaric acid, in the presence of an acidic substance and in an aqueous solution of a volatile base as sole emulsifying agent, said acidic substance being selected from the group consisting of natural resins containing resin acid and having an electric resistance of at least 10<sup>11</sup>Ω·cm., synthetic resins containing a carboxyl radical and having an electric resistance of at least 10<sup>11</sup>Ω·cm., alicyclic compounds having a carboxyl radical, aliphatic carboxylic acids, aromatic carboxylic acids and acid anhydrides of said carboxylic acids; applying a film of said emulsion onto said conductive support and drying said film for a time sufficient to evaporate substantially all of said volatile base.

2. The method of claim 1 in which the volatile base is a member selected from the group consisting of ammonia, a lower aliphatic amine, an aromatic amine, morpholine and piperidine.

5 3. The method of claim 1 wherein the emulsifying step comprises mixing an organic solvent solution of said resinous binder and said acidic substance and an aqueous solution of said volatile base.

4. An electrophotographic copying material comprising an electro-conductive support and having applied thereon a photoconductive film comprising a resinous binder having dispersed therein a photoconductive substance selected from the group consisting of zinc oxide, titanium oxide, cadmium sulfide and zinc selenide, said resinous binder consisting of a copolymer of at least one member selected from the vinyl monomer group consisting of glycidyl acrylate, glycidyl methacrylate, hydroxyethyl methacrylate, hydroxyethyl acrylate, hydroxypropyl methacrylate, hydroxypropyl acrylate, 5-hydroxypentylvinyl ether ( $\text{CH}_2=\text{CHOCH}_2\text{CH}_2\text{CH}_2\text{CH}_2\text{CH}_2\text{OH}$ ) with at least one member selected from the monomer group consisting of styrene, alkyl acrylate, alkyl methacrylate, acrylonitrile, vinyl chloride, vinylidene chloride, vinyl acetate, acrylic acid, methacrylic acid, crotonic acid, itaconic acid, maleic acid and fumaric acid, and being one which is water-emulsifiable in the presence of an acidic substance and a volatile base to form an emulsion stable upon mixing with said photoconductive substance, said film having dispersed therein an acidic substance selected from the group consisting of natural resins containing resin acid and having an electric resistance of at least 10<sup>11</sup>Ω·cm., synthetic resins containing a carboxyl radical and having an electric resistance of at least 10<sup>11</sup>Ω·cm., alicyclic compounds having a carboxyl radical, aliphatic carboxylic acids, aromatic carboxylic acids and acid anhydrides of said carboxylic acids, said film having been dried for a time sufficient to evaporate substantially all of said volatile base.

10 5. The article of claim 4 which also contains a small amount not exceeding 0.5% per total weight of said photoconductive film of a volatile base.

6. The article of claim 4 wherein said photoconductive film contains a volatile base selected from the group consisting of ammonia, methylamine, dimethylamine, trimethylamine, ethylamine, diethylamine, triethylamine, propylamine, butylamine, hexylamine, ethylenediamine, arylamine, morpholine, piperidine and hydrazine, said volatile base being present in said film within a range not exceeding 0.5% per total weight of said photoconductive film.

#### References Cited

##### UNITED STATES PATENTS

|    |            |         |                  |        |
|----|------------|---------|------------------|--------|
| 55 | Re. 25,444 | 9/1963  | Kucera           | 96—1   |
|    | 2,997,387  | 8/1961  | Tanenbaum        | 96—1   |
|    | 3,159,483  | 1/1964  | Behmenhey et al. | 96—1   |
|    | 3,160,503  | 12/1964 | Cady             | 96—1   |
|    | 3,245,786  | 4/1966  | Cassiens         | 96—1   |
| 60 | 3,248,217  | 4/1966  | Shulman          | 96—1   |
|    | 3,261,709  | 7/1966  | Shulman          | 117—34 |
|    | 3,307,942  | 3/1967  | Cole             | 96—1.8 |
|    | 3,409,575  | 11/1968 | Cole             | 260—27 |
|    | 3,345,162  | 10/1967 | McFarline        | 96—1.8 |
| 65 | 3,489,559  | 1/1970  | Clark            | 96—1.5 |

#### OTHER REFERENCES

Fundamental Principles of Polymerization by D'Alelio, Wiley & Sons, New York, N.Y., 1952, p. 202.

JOHN C. COOPER III, Primary Examiner

U.S. Cl. X.R.